

Sept. 28, 1954

E. WAINER

2,690,409

BINARY COATING OF REFRACTORY METALS

Filed July 8, 1949

*FIG. 1*



*FIG. 2*



*Inventor*  
Eugene Wainer

*by* *Law Firm of Charles Abbott* *Atty's*

## UNITED STATES PATENT OFFICE

2,690,409

## BINARY COATING OF REFRACtORY METALS

Eugene Wainer, Cleveland, Ohio, assignor to  
 Thompson Products, Inc., Cleveland, Ohio, a  
 corporation of Ohio

Application July 8, 1949, Serial No. 103,632

4 Claims. (Cl. 148—31.5)

1

The present invention relates to a method of coating refractory metal articles to enhance their resistance to high temperature and corrosive atmospheres. The present invention specifically relates to the manufacture of coated refractory metal turbine buckets for use in jet turbines and the like.

Turbo-jet engines or the like are usually provided with an axial flow turbine operated by exhaust gases which drive a blower furnishing air to the burners. Such turbines operate at extremely high temperatures, and one of the major difficulties encountered in the manufacture of jet turbines has been the provision of suitable material for bucket blades which can withstand the effect of such high temperatures. The turbine bucket will normally be exposed to temperatures in the range of from 1600° to 2000° F. and the bucket must have sufficient strength, toughness, creep resistance, and resistance to the corrosive atmosphere present to enable the bucket to operate efficiently without deformation or corrosion.

In addition to turbine buckets, articles produced by the present invention may be employed under conditions of higher temperature and lower stress than exist in a gas turbine bucket. One such application occurs in nozzle diaphragm vanes in gas turbines which must withstand very severe conditions of temperature and thermal shock but at a relatively lower stress.

One refractory metal which exhibits excellent properties of strength, toughness and creep resistance at elevated temperatures is molybdenum. However, metallic molybdenum itself cannot be used. The trioxide of molybdenum, which is formed under the oxidizing conditions present in the turbine, sublimes at a temperature of about 1463° F. at an extremely rapid rate. This phenomenon gives rise to a characteristic smoking when bodies of molybdenum are heated to temperatures above 1463° F., resulting in the complete disappearance of the molybdenum within a matter of minutes. Another refractory metal which might be used for turbine bucket bodies is tungsten, even though it has a relatively high density.

To overcome this difficulty, I have herein provided a process for coating refractory metal such as molybdenum to provide thereon a tough, corrosion-resistant coating impervious to the effect of oxygen and other gases.

It is then an object of the present invention to provide a method for coating refractory metals such as molybdenum to provide an extremely corrosion resistant surface thereon.

2

Another object of the present invention is to provide a method for coating refractory metals which yields a firm bond to the refractory surface and makes it impervious to the effects of operation under conditions of high stress and high temperatures.

A further object of the invention is to provide a coated molybdenum article, such as a turbine bucket, capable of operation within a turbine engine for extended periods of time without deterioration.

In the process of the present invention, the refractory metal is coated with a metal selected from the group consisting of silicon, aluminum, and zirconium and the coating is subsequently reacted with another element to produce a binary coating. The coating and reaction steps may be carried out concurrently, or the refractory metal may be given a primary coat of silicon, aluminum or zirconium and subsequently reacted with the second element, which is preferably selected from the group consisting of the elements in groups III, IV or V of the periodic table.

The element which is to be reacted with the primary coating is one whose ionic size is close enough to the ionic size of the primary metal coating to allow the elements to be mutually soluble with each other in the solid state, and thus increase the rate of intermetallic compound formation. Such intermetallic compounds per se or the compounds formed with the base metal then have a size which approximates the atomic spacing in the lattice of the base metal. The primary coating inherently leaves microscopic voids, tunnels or weak spots in the surface of the article, thus decreasing its ability to withstand corrosion. By reacting the primary coating with a second element of the type mentioned, it is believed that the voids in the atomic spacing of the single metal are filled by the reaction with the second element, thus making the layer much less permeable. The reaction with the second element depends primarily upon the spacing in the crystal lattice of the primary coating. Where the primary coating is silicon, the secondary element may be titanium, zirconium, boron, aluminum, nitrogen, or carbon. In the case of aluminum, a primary coat of this metal may be further reacted with zirconium, titanium, chromium, boron, tin, and nickel. Where zirconium is used as the primary coat, the subsequent reaction may be carried out with aluminum, boron, carbon, silicon, titanium, and nitrogen.

The compounds resulting from the reaction of

the second named elements with the primary coating are complex intermetallic compounds which exhibit the property of forming an extremely firm bond to the surface of the refractory metal. It is believed that this firm bond results from the closure of voids in the atomic lattice of the base metal, but the present invention is in no way limited to the correctness of the given theory.

The coating process of the present invention may be most conveniently carried out in a vapor phase deposition system of the type described in a copending application Serial No. 98,272, filed June 10, 1949 by myself and Robert A. Kempe. In that application, there is described a method for coating refractory metals wherein a decomposable compound, preferably a halide, of the coating metal is carried into a reaction zone in a stream of hydrogen and therein decomposed to form a layer of substantially pure metal on the surfaces of the refractory metal. Deposition of the coating metal compound, as discussed in this previous application, is the result of several factors. Some of the compound is probably decomposed by the high temperatures, on the order of 1600° to 2300° F. present in the coating zone. Another portion of the decomposable coating compound is reduced by the presence of the hydrogen atmosphere in which the compound is introduced. Another reaction which occurs is the metathetical reaction between the coating metal compound and the molybdenum wherein the coating metal is deposited on the molybdenum with the formation of a volatile molybdenum compound in the exchange reaction.

The decomposable compound employed in the primary coating step is preferably a halide, for example silicon tetrachloride, trichlor silane, silicon tetrabromide, tribromo silane, silicon tetr碘ide, aluminum chloride, aluminum bromide, aluminum iodide, zirconium chloride, zirconium bromide, or zirconium iodide. Where the coating metal compound exists normally in the liquid state, as is in the case of silicon tetrachloride, the coating metal compound may be introduced into the heated reaction zone by merely passing a stream of hydrogen gas through a liquid pool of the compound so that vapors thereof are carried by the hydrogen into the reaction zone. Where the coating metal compound is normally solid, the hydrogen gas may be passed over a heated source of the compound in powder form to carry it into the reaction zone.

In reacting the primary coating with the second element, a decomposable compound capable of yielding the second element is introduced into the reaction zone either prior to, during, or after the deposition of the primary coating. Typical decomposable compounds which may be used in this connection are titanium tetrachloride, titanium tetrabromide, chromium chloride, nickel chloride, boron chloride, and tin chloride. Where the primary metallic coating is to be carburized, i. e., reacted with carbon, a carburizing gas is introduced into the reaction zone. Any common carburizing gas such as natural gas, carbon monoxide, ethane, propane, butane, and benzene may be used, or the carburizing operation may be carried out in carburizing packs, or in liquid baths.

Where the primary coating is to be nitrided, i. e., reacted with nitrogen, ammonia gas is preferably introduced into the reaction chamber to react with the primary coating. In addition to

ammonia gas, various decomposable cyanides may be employed.

The reaction conditions in the coating zone include temperatures from 1600° to 2300° F. and preferably from 1700° to 2100° F. and reaction times ranging from 4 to 24 hours depending upon the penetration required. Normally, the depth of the primary coating will be on the order of about 0.0003 to about 0.003 inch.

Where silicon is used as the primary coating metal, the outermost layer is substantially pure silicon, the next layer is probably a molybdenum-silicon compound having a relatively high silicon content, possibly  $MoSi_2$ , while the innermost layer produced by the coating process is essentially a molybdenum-silicon compound having a high molybdenum concentration, such as  $Mo_2Si$  together with solid solutions of molybdenum and silicon. This type of structure is one which is stable at high temperatures, and provides an excellent intimate bond with the molybdenum base. The reaction with the second element of the type mentioned above enhances the properties of the coating by filling up the microscopic voids and weak spots, resulting in a substantial increase in stability and resistance to high temperature oxidation.

A further description of the present invention will be made in connection with the attached sheet of drawings in which:

Figure 1 is a flow sheet showing in general the various stages of the coating process; and

Figure 2 is a drawing of a photomicrograph taken as a magnification of 500X showing the crystal structure of a molybdenum article coated in accordance with the present invention.

As shown on the drawings:

Reference numeral 10 denotes a supply of purging gas, which is preferably an inert gas such as nitrogen, argon, neon, helium or the like which is passed into a purification zone 11 where moisture and other contaminants are removed. The purification zone 11 may consist of a supply of liquid sulfuric acid through which the purging gas is bubbled. The purified gas is next introduced into a heated furnace 12 which surrounds a furnace tube 13, control of the gas flowing into the furnace tube being controlled by means of a valve 14.

Disposed within the furnace tube 13 are a plurality of boats 15 which carry a number of turbine buckets 16 or other articles composed of a refractory metal such as molybdenum. These articles are normally preshaped into their desired form, and worked at temperatures below the recrystallization temperature of the metal, to enhance its physical properties. The temperature of the furnace 12 is regulated between 1600 and 2300° F., with 1700 to 2100° F. being a preferred range.

A supply of hydrogen gas 17 is provided for introduction into the furnace tube 13. Prior to its introduction into the furnace tube 13, the hydrogen gas is dehydrated and purified by means of various desiccants such as, for example, packed columns of silica gel, calcium chloride, or liquid sulfuric acid in a purification stage 18. The flow of the hydrogen gas into the furnace tube 13 is controlled by means of a valve 19. A second source of hydrogen gas 20 and its purification stage 21 is also provided to act as a carrying medium for the coating compounds. A source of the primary coating compound A, normally a decomposable halide, is maintained in a zone 22. A source of a compound, B, of the second re-

active element which may be one of the metals given previously, or a carburizing or nitriding gas is indicated at zone 23. Flow into the zones 22 and 23 is regulated by means of the respective valves 24 and 25 while flow of hydrogen gas containing the coating compounds is regulated by means of the valves 26 and 27 at the exit of stages 22 and 23. In this arrangement, either of the coating compounds may be introduced separately into the reaction zone or the introduction of both compounds may be made simultaneously.

Initially, the furnace tube 13 is purged by means of the purging gas 10 to rid the furnace chamber of moisture and oxygen or other undesirable contaminants. Thereupon, the hydrogen and the coating metal compound which it carries is introduced into the furnace tube 13, where it contacts the molybdenum article 16 for periods of time ranging from 4 to 24 hours. Excess hydrogen is vented from the furnace tube by means of tube 28. The molybdenum articles 16 are maintained in the furnace tubes 13 until a coating having a thickness of approximately .0003 to .003 inch is produced on the article.

In Figure 2, there is shown a drawing of a photomicrograph of a molybdenum turbine bucket produced by simultaneous vapor deposition of silicon and titanium for a period of eight hours at a temperature of 2000° F. As illustrated in that drawing, the body of the article consists of rather large crystals of molybdenum 29 having an overlying layer of silicon 30. Immediately above the silicon layer 30 is a layer 31 of indeterminate composition, which is probably a complex mixture of molybdenum, titanium and silicon in the form of various intermetallic compounds. The uppermost layer 32 is a mixture of titanium and silicon compounds of these two elements. This structure has been found capable of withstanding operation in a gas turbine operating at temperatures estimated at 1600° to 1800° F. for periods in excess of 100 hours without apparent deterioration.

From the foregoing, it will be appreciated that I have herein provided a process for coating refractory metals which are in themselves incapable of withstanding the corrosive effect encountered in the operation of a gas turbine.

The coatings produced in accordance with this invention are integrally bonded to the base metal and cannot be stripped mechanically from the body metal, as is the case of coatings applied by electroplating or dipping. Further, the coatings are inert with respect to the molybdenum base metal and show no evidences of reaction with the base metal after the original deposition.

The vapor phase deposition processes described herein have complete "throwing power" i. e., a uniform coating can be deposited over the entire surface of the article regardless of corners, grooves or other irregularities in the surface of the article. This is not true of other types of coating procedures.

It will be understood that modifications and variations may be effected without departing from the scope of the novel concepts of the present invention.

I claim as my invention:

1. The method of providing a corrosion resistant surface on a molybdenum article which comprises depositing a layer of silicon on said article, and nitriding the silicon layer.
2. A molybdenum body having a corrosion resistant outer layer of nitrided silicon thereon.
3. The method of providing a molybdenum body with a corrosion resistant coating, which comprises depositing on the surface of said body a layer consisting essentially of an element selected from the group consisting of silicon and zirconium, and reacting the selected element in said layer with a different element selected from the group consisting of silicon, zirconium, titanium, boron, aluminum and nitrogen to form a binary coating on said body, said coating being integrally bonded to the molybdenum body.
4. A molybdenum body having an outer corrosion resistant coating thereon consisting essentially of the reaction product of an element selected from the group consisting of silicon and zirconium with a different element selected from the group consisting of silicon, zirconium, titanium, boron, aluminum and nitrogen, said coating being integrally bonded to the molybdenum body.

40 References Cited in the file of this patent

UNITED STATES PATENTS

| Number    | Name                  | Date          |
|-----------|-----------------------|---------------|
| 1,551,333 | Schroter et al. ----- | Aug. 25, 1925 |
| 1,929,252 | Morris -----          | Oct. 3, 1933  |
| 2,096,924 | Schwartzkopf -----    | Oct. 26, 1937 |
| 2,235,504 | Rennie -----          | Mar. 18, 1941 |
| 2,294,562 | Kingston -----        | Sept. 1, 1942 |

FOREIGN PATENTS

| Number  | Country      | Date          |
|---------|--------------|---------------|
| 842,981 | France ----- | June 22, 1939 |

OTHER REFERENCES

55 Metals Handbook, 1939 edition, pages 1054, 1055, 1074, 1090. Published in 1939 by the American Society for Metals.